

J. S. WEYL.

PROCESS OF FINISHING THE SURFACE OF COATED CALENDERED PRINTING PAPER.

APPLICATION FILED DEC. 31, 1913.

1,125,232.

Patented Jan. 19, 1915.



Fig. 1.



# UNITED STATES PATENT OFFICE.

JULIUS S. WEYL, OF ELKINS PARK, PENNSYLVANIA.

## PROCESS OF FINISHING THE SURFACE OF COATED CALENDERED PRINTING-PAPER.

1,125,232.

Specification of Letters Patent.

Patented Jan. 19, 1915.

Application filed December 31, 1913. Serial No. 809,627.

To all whom it may concern:

Be it known that I, JULIUS S. WEYL, a citizen of the United States, residing at Elkins Park, Montgomery county, State of Pennsylvania, have invented certain new and useful Improvements in Processes of Finishing the Surface of Coated and Calendered Printing-Paper, of which the following is a full, clear, and exact description, reference being had to the accompanying drawings, forming a part of this specification.

My invention relates to the preparation of the surface of printing paper to better adapt it, in smoothness, evenness of surface and absence of shine or gloss, to relief printing of fine plate engravings including especially such as printed from photo-mechanical half tone plates.

In the preparation of the surface of printing paper for relief printing such as the production of fine half tone engravings, a so-called coated paper must be employed to obtain the required smoothness of surface, such coating being effected by the agency of a mechanically-rotated brush application of a mixture consisting of a finely ground mineral substance such as English clay, with casein, glue or the like, and then dried and calendered; but such coated paper, even when the calendering is applied with carefully adjusted pressure, has imparted to it a surface which though smooth, is so glossy that it reflects light, which not only obstructs a full and proper view of the engraved picture, but is injurious to the eyes of the reader. To avoid this objectionable glossy effect of coated and calendered printing papers it has been attempted to "dull" it, either by admixing a certain proportion of ground barium sulfate crystals with the clay, in the coating mixture, or by minimizing the usual calendering effect by adjustment of the pressure of the rolls; but neither method satisfactorily accomplishes the result sought, because while producing a surface free from excessive glare an uneven surface is frequently the result, making uniform plate printing impossible.

To overcome the objections stated and to produce a coated printing paper having a fine smooth and even surface and free from gloss, I have discovered a method which is simple and yet effective and which consists essentially in subjecting the paper in the

coated condition after drying, and with or without calendering, and while properly supported and in motion, to the action of a suitably applied sand blast, somewhat after the method of mechanically etching 60 cut glass.

In the accompanying drawings I have illustrated mechanical means suitable for applying the sand blast to the paper to be treated.

In said drawings Figure 1 is a plan view with the closing cover and paper-supporting plate removed, and Fig. 2 a side elevation of the complete device partly in section.

Referring to said drawings, 1 indicates a 70 suitable inclosing frame, the rectangular open top of which supports a like shaped flat frame 9<sup>a</sup>, and upon the latter is rested a like shaped covering frame 12 which is closed except at its center 12<sup>a</sup>, and between 75 said cover 12 and frame 9<sup>a</sup> is mounted a paper-supporting board 11 which is of the full width of the roll of paper to be treated and somewhat less than the width of the said parts 1, 9<sup>a</sup> and 12. Mounted within 80 the inclosing frame 1 and extending through to its opposite side walls is a horizontally-disposed tube 3 which serves as a conduit for compressed air derived from any adjacent source of supply.

The tube 3, for a distance within the inclosing frame is provided with an elongated narrow discharge nozzle 3<sup>a</sup>, the apex or top of which projects upward and into a pressure and sand chamber 4 which may be in 90 the form of a square plate with a central depression and edge flanges 5, and upon the latter rests a flat cover plate 6, having a central elongated aperture disposed immediately over the mouth of the nozzle 3<sup>a</sup>, and 95 in said aperture in the plate 6 is mounted a vertically disposed sand-discharge nozzle 8, which as seen in top view in Fig. 1, has a discharge end in the form of an elongated slit, slightly less in length than the width 100 of the roll of paper to be treated. In the plate 5 are two series of perforations 6<sup>a</sup> 6<sup>b</sup> operating as sand holes, and arranged in parallelism with each other and with the sand discharge nozzle 8 and on each side 105 thereof.

Resting with its base on the plate 5 is a hopper 7, of suitable shape to accord with the frame. The top edges of the inclined walls of the hopper rest on the inner edges 110

of the element 9<sup>a</sup> and within the inclosing frame 1. Within the hopper 7 is a sand screen 9 through which the extreme top of the elongated sand nozzle 8 projects. 5 Within each of the elements 9<sup>a</sup>, 9<sup>a</sup> are loosely mounted a pair of freely rotatable guide rollers 10, 10 and on the inlet side of the supporting frame 1 and within the same is mounted a freely rotatable paper 10 supporting and guiding roller 10<sup>a</sup>. On the middle side of the apparatus is located a stand 13 adapted to support a length of paper to be treated, rolled up on a rotatable holder 14; and on the opposite 15 side of the apparatus is a like stand 13<sup>a</sup> supporting a take-up roller 15 driven by a pulley 16, which may be actuated by suitable means such as an electric motor, indicated at 17. In operating the device to 20 carry out my process, I have obtained successful results by employing a fine quality of sand commonly used for etching work, and compressed air pressure, at the discharge nozzle, of one and three quarters to 25 five pounds, with the discharge end of the nozzle 8 at a distance of five or six inches from the surface of the paper and discharging at right angles thereto; though doubtless all these proportions may be varied 30 depending on the relative sizes of the various elements of the described means employed; while the speed of the take-up roller, which governs the time of exposure of the paper to the blast, will be found 35 satisfactory if it draws the paper 18 continuously and steadily across the blast at the rate of two to six feet per minute, guided in its delivery in a horizontal plane by the freely rotatable guide rollers de- 40 scribed, and supported from the rear side by the plate 11 which is of the width of the roll of paper and is supported by its opposite ends in suitable openings in the frame element 9<sup>a</sup> before mentioned. 45 The initial charge of sand is supplied to the hopper, above the screen, by removing the cover 12; while any powder therefrom or that negligible quantity thereof which is from the paper by action of the sand blast 50 therein, is blown out of the top opening 12<sup>a</sup> of the cover 12; the sand from the blast, after acting on the paper, drops back through the screen 9, thence through the perforations 6<sup>a</sup> in the plate 6 and thence

into the sand chamber 4 of the air-nozzle 55 plate.

In applying my novel method for treating coated and calendered printing papers to attain the desired results stated, it will be observed that the exposure of the paper to 60 the reducing action of the blast is a limited one because applied to a constantly moving and hence constantly changing portion of the roll, and is very effective to remove the gloss from the surface without the slightest 65 injury to it; while the tautness of the paper effected by the take-up roller, maintained in a guided horizontal plane, by the guide rollers and the plate against which the rear side of the paper contacts in its let off motion, permits the reducing action stated to 70 produce its results under conditions to effect a perfectly even as well as smooth surface of the paper so treated.

Having thus described my invention, I 75 claim:—

1. The process of treating coated calendered printing paper to remove the gloss, while maintaining its calendered smoothness and evenness of surface, which consists in applying thereto the reducing action of a suitably applied sand blast, substantially as described.

2. The process of treating coated and calendered printing paper for the purposes described, which consists in subjecting the printing surface of the paper, under horizontally guided motion, to the action of a sand blast discharging in the path of the moving paper.

3. The process of treating coated and calendered printing paper for the purposes of removing its gloss without affecting its calendered smoothness, and simultaneously imparting to it an even surface, which consists 95 in imparting guided horizontal motion to the paper against a like supporting surface and in the path of a sand blast discharging transversely to the direction of the movement of the paper.

In testimony whereof I have hereunto affixed my signature this 19th day of December, A. D. 1913.

JULIUS S. WEYL.

Witnesses:

H. B. COURTER,  
S. C. STEIN.